

# UNITED STATES PATENT OFFICE.

CARL ROESSLER, OF HAMBURG, GERMANY.

## METHOD OF MANUFACTURING LEATHER SUBSTANCES.

1,192,460.

Specification of Letters Patent. Patented July 25, 1916.

No Drawing.

Application filed August 28, 1913. Serial No. 787,143.

To all whom it may concern:

Be it known that I, CARL ROESSLER, manufacturer, a subject of the German Emperor, and residing at Hamburg, Germany, have 5 invented certain new and useful Improvements in Methods of Manufacturing Leather Substances, of which the following is a specification.

The present invention relates to a method 10 of manufacturing leather substances which can be used, for instance, as floor covering material or a material for making jointless floors.

The method consists essentially in grinding 15 leather or leather waste alone or mixed with other fibrous substances such as asbestos, simultaneously with non-fibrous substances of granular nature and in adding a suitable binding agent thereto.

20 In carrying out the method, leather or leather waste of any kind, tanned leather as well as untanned leather, may be utilized.

As non-fibrous substances, mineral and 25 also organic substances, come, for instance into consideration. The leather, the leather waste or its or their mixtures with asbestos or the like are ground together with non-fibrous substances in a suitable grinding device, the fibrous nature of the leather being 30 preserved and the product thus obtained being made into a thick paste with a suitable binding agent.

This paste can be applied directly upon a suitable base and thus be used, for instance, 35 for the production of jointless floors. It can, however, be also made into plates or slabs of any thickness and size by using pressure.

Example I: 100 kilograms of leather 40 waste are ground with 20 kilograms of coarse asbestos threads, 162 kilograms of magnesium oxid, 10 kilograms of kieselguhr and 15 kilograms of metal oxid, or earthen colors and the product obtained is made into 45 a thick paste with a 25% addition of a solution of magnesium sulfate. This paste can be used either as a jointless floor or, for instance, be made into slabs under hydraulic pressure.

50 Another manner of carrying out the method of the present invention consists, after having ground the leather or leather waste with the non-fibrous substances, in

adding to the product thus obtained, a small percentage of glycerin and making these 55 substances into a thick paste by means of a binding agent such as linseed oil.

Example II: 100 kilograms of leather waste are ground with 20 kilograms of asbestos, 27 kilograms of casein and 15 kilograms of metal oxid or earthen colors, 150 grams of glycerin are added thereto and the product thus obtained is made into a thick paste by adding 7 kilograms of pulverulent slaked lime with 30 liters of linseed oil. 65

Finally, for the manufacture of the substances in accordance with the invention, a binding agent constituted by tar oils or mineral oils, may also be used and which may contain mineral substances such as 70 silicates and the like. This kind of substances is very appropriate as floor covering material for drill halls, circuses and the like.

The leather substances manufactured in 75 accordance with the present invention have, in comparison with the known substances, advantages in various respects. They are thus characterized by a greater elasticity and are more resisting mechanically as well 80 as against moisture. They are therefore well washable. Furthermore they can be treated in any manner for instance, they can be sawed, cut, impressed and so on, without losing solidity or disintegrating. 85

I claim:

1. The method of manufacturing leather substances, which comprises grinding leather waste with asbestos, magnesium oxid, kieselguhr and a color to obtain a triturated 90 fibrous product, and then adding about one-fourth part of magnesium sulfate.

2. The method of manufacturing leather substances, which comprises grinding 100 95 kilograms of leather waste with 20 kilograms of asbestos, 162 kilograms of magnesium oxid, 10 kilograms of kieselguhr and 15 kilograms of coloring material, and mixing the resulting product with magnesium sulfate sufficient to bind the mass. 100

In testimony whereof, I affix my signature in the presence of two witnesses.

CARL ROESSLER.

Witnesses:

WOLDEMAR HAUPT,  
ARTHUR SCHROEDER.